

# UNITED STATES PATENT OFFICE.

WILLIAM R. D. HALL, OF NARBERTH, PENNSYLVANIA, ASSIGNOR TO S. FEATHER COMPANY, A CORPORATION OF DELAWARE.

## PROCESS FOR SPINNING ARTIFICIAL-SILK WASTE.

1,340,044.

Specification of Letters Patent. Patented May 11, 1920.

No Drawing.

Application filed June 26, 1918. Serial No. 242,111.

To all whom it may concern:

Be it known that I, WILLIAM R. D. HALL, a citizen of the United States, residing at Narberth, in the county of Montgomery and State of Pennsylvania, have invented new and useful Improvements in Processes for Spinning Artificial-Silk Waste, of which the following is a specification.

It is a well-known fact that the use of artificial silk waste has been tremendously restricted, especially in the use of the same with respect to yarn, etc., for the reason that, contrary to real silk waste, the fiber of the artificial silk waste cannot be spun out to a very fine thread *i. e.* finer than about 20,160 yards to the pound, due to the smooth and slippery nature of the fiber.

I have now invented a process whereby yarn may be produced, having as its base artificial silk waste, which yarn may be finer by far than the yarn heretofore produced from artificial silk waste.

I accomplish the above by adding to artificial silk waste 18 per cent. of real silk waste, subsequently mixing and intertwining the fibers one with the other and then treating the whole with 5 per cent. of lard oil. This mixture is then spun out and the results desired are obtained.

It will be noted, however, that the silk waste must nearly approximate the artificial silk waste in luster so that the small addition of real silk waste to the artificial silk waste does not, to an appreciable extent, detract from the luster of the finished yarn, which luster, as is known, is very brilliant in the yarn derived from artificial silk waste.

It will also be noted that not alone do I accomplish the production of a finer yarn by the above process, but after the yarn has been manufactured a very unique effect may be obtained due to the fact that the

silk waste is an animal product and the artificial silk waste is a vegetable fiber. The 45 result above referred to is reached by treating the yarn with a dye which does not act upon vegetable fiber, or vice versa upon animal fiber. It will be seen that by using either one of these dyes, one of the fibers 50 will retain its natural color whereby a very novel effect is produced. On the other hand, the whole may be treated with what is known as a union dye to color the same a constant shade.

It will be noted that by summing up the above results, in combining the artificial silk waste to the real silk waste it is possible to spin the artificial silk waste to a much finer thread than if the same had been used 60 alone.

The addition of the real silk waste to the artificial silk waste does not noticeably detract from the luster of the yarn produced from the latter.

Novel effects can be obtained in dyeing by the use of a dye which may act either upon animal fibers or vegetable fibers, and the same result can be obtained in dyeing the finished product as though no real waste 70 had been used.

Having described my invention, what I claim is:—

1. The process of producing yarn of very fine diameter from artificial silk waste, said 75 process consisting in mixing artificial silk waste with real silk waste in the proportion of about 82 per cent. of the former and 18 per cent. of the latter, treating the mixture with oil, and spinning such treated mixture. 80

2. In the production of yarn, the mixture of artificial silk fiber and real silk waste of approximately the same luster, treating the whole with oil and spinning such mixture.

WILLIAM R. D. HALL.